# EUROPEAN PATENT APPLICATION

(11) **EP 4 614 534 A1**
(43) Date of publication of application: **10.09.2025**
(21) Application number: 23884920.2
(22) Date of filing: 31.10.2023
(51) Int. Cl.: H01F 1/34, H01F 17/00, H01F 41/04

(54) **MAGNETIC MATERIAL AND MULTILAYER INDUCTOR COMPRISING SAID MATERIAL**

(30) Priority: 02.11.2022 CN 202211360830
(71) Applicant: Steward (Foshan) Magnetics Co., Ltd., Foshan, Guangdong 528322 (CN)
(72) Inventor: ZHANG, Jacken, Foshan, Guangdong 528322 (CN); CHIANG, Yeat Shing, Foshan, Guangdong 528322 (CN); PANG, Wenshan, Foshan, Guangdong 528322 (CN)
(74) Representative: Lind Edlund Kenamets Intellectual Property AB
(86) International application number: PCT/CN2023/128371
(87) International publication number: WO 2024/093990

(57) **Abstract**

The present invention relates to a magnetic material and a multilayer inductor including said magnetic material. Specifically, the magnetic material is formed by sintering an oxide used for forming a ferrite material and a doping oxide, and is characterized in that the magnetic material has a crystal structure, the doping oxide is distributed on grain boundaries of the crystal structure in a doped phase, and the content of the doping oxide is 5 wt% or less based on the total weight of the magnetic material. According to the present invention, the magnetic material can improve the grain boundary resistance at low sintering temperatures and can increase the impedance of magnetic materials.

## Description

### TECHNICAL FIELD

The present invention relates to the field of electronic devices, and relates specifically to a multilayer inductor structure for a power application. Specifically, the multilayer inductor structure is used for voltage-to-current conversion for power transmission, impedance matching for data transmission and processing, and filtering of electromagnetic interference.

### BACKGROUND

As one kind of passive device, inductors may generally be classified into: winding-type inductors, which are manufactured by winding a coil around a ferrite core and forming electrodes at both ends thereof; and multilayer-type inductors, which are manufactured by printing an internal electrode on a magnetic layer or a dielectric layer and then stacking magnetic layers or dielectric layers.

In recent years, due to the development of thick film printing processes and LTCC materials, there has been a need for further miniaturization of passive devices such as resistors, capacitors, and inductors. As a solution for a miniaturized and low-cost optimal SMT inductor in a small circuit board, multilayer-type inductors are gradually gaining dominance compared to winding-type inductors.

In general, a multilayer inductor includes a multilayer body formed of a plurality of magnetic sheets having internal electrodes of coil patterns formed on one surface thereof.

A ferrite material is generally used as a body material or a magnetic core material, and a metal such as silver is generally used as an electrode material. When an inductor core is co-sintered with a metal track such as silver to obtain an integral structure, the sintering temperature of the magnetic core is usually 900°C or lower, which is lower than the melting point of silver (approximately 963°C). Therefore, an additional composition needs to be added, which will reduce the magnetic performance of the core. In addition, high core resistance is needed to insulate silver conductive traces, which will also reduce the magnetic performance.

There are many techniques for improving such a magnetic material in the prior art. For example, CN112341179A proposes a high-frequency manganese-zinc ferrite material, which includes a main crystalline phase and a doped crystalline phase, wherein the doped crystalline phase is uniformly doped in a grain boundary and the main crystalline phase. CN107004478A proposes a magnetic material, which includes a magnetic phase and a grain boundary phase, wherein the grain boundary phase includes at least one metal and has a melting temperature lower than that of the magnetic phase. CN106486236A proposes a magnetic core material, which includes a crystalline phase and an insulating film, wherein the insulating film is formed surrounding the crystalline phase.

However, the above-mentioned techniques provide very little improvement in terms of the magnetic properties or magnetic flux density of the magnetic core material. Therefore, there is still a need in the art to develop techniques for improving the magnetic properties or magnetic flux density of magnetic core materials.

### SUMMARY OF THE INVENTION

### Technical Problem

In view of the above, the present invention relates to providing a magnetic material for a magnetic core of a multilayer inductor, and grain boundary resistance at low sintering temperatures can be improved and the proportion of a non-magnetic material can be minimized by adding a specific inorganic additive to the magnetic material to help the formation of magnetic powder.

The inventors of the present invention found that the sintering of ferrite materials can be promoted by means of dissolution promoting elements such as Si, Bi, and Ca, wherein Si can promote low-temperature firing of ferrite while high-resistance precipitates can be formed at grain boundaries; Bi can form low-melting point phases to promote ferrite particle growth, and at the same time, by sintering at a reduced temperature, a fired particle size is reduced, grain boundary resistance is increased, the proportion of Fe is reduced, and the generation of Fe²⁺ in the ferrite is reduced; Ca can also achieve the purpose of increasing the grain boundary resistance and simultaneously promoting dissolution together with elemental Si, so as to achieve the purpose of reducing the firing temperature; and resistance can be improved overall by increasing the content of high-resistivity Ni, thereby completing the present invention.

Another aspect of the present invention relates to a multilayer inductor, and excellent magnetic properties or magnetic flux density can be implemented by improving a magnetic core material thereof.

### Technical Solution

According to a first aspect of the present invention, a magnetic material for a magnetic core of a multilayer inductor is provided, the magnetic material being formed by sintering an oxide used for forming a ferrite material and a doping oxide, and being characterized in that the magnetic material has a crystal structure, the doping oxide is distributed on grain boundaries of the crystal structure in a doped phase, and the content of the doping oxide is 5 wt% or less based on the total weight of the magnetic material.

In an implementation, the doping oxide comprises silicon dioxide, bismuth oxide, optionally calcium oxide, or a combination thereof.

In an implementation, the magnetic material comprises a ferrite material forming grains in the crystal structure, with Fe₂O₃ as a main body material.

In addition, in a specific implementation, the ferrite material further comprises at least one selected from Mn₃O₄, NiO, CuO, and ZnO as an additive.

In a specific embodiment, the ferrite material is an NiCuZn ferrite, with a chemical formula of NiCuZnFe₂O₄.

In a specific implementation, based on the total weight of the oxide used for forming the ferrite material, the content of Fe₂O₃ may be 62 wt% to 65 wt%; the content of NiO may be 10 wt% to 13 wt%; the content of ZnO may be 19 wt% to 22 wt%; the content of CuO may be 2 wt% to 5 wt%; and the content of Mn₃O₄ may be 0 wt% to 1 wt%, preferably 0.1 wt% to 1 wt%.

In an implementation, based on the total weight of the magnetic material and the total weight of the oxide used for forming the ferrite material, the content of the doping oxide is preferably as follows: SiO₂: 0.01 wt% to 0.15 wt%; Bi₂O₃: 0.1 wt% to 3 wt%; and CaO: 0 wt% to 1.5 wt%.

According to another aspect of the present invention, a multilayer inductor is provided, which comprises a plurality of magnetic layers and metal electrode tracks formed on the magnetic layers, the magnetic layers comprising the magnetic material for the magnetic core of the multilayer inductor of the present invention.

In an implementation, the metal electrodes comprise silver (Ag), platinum (Pt), palladium (Pd), copper (Cu), gold (Au), nickel (Ni), or an alloy thereof, or a composite thereof.

According to a further aspect of the present invention, a method for preparing the magnetic material of the present invention is provided, the method comprising the following steps:
(a) mixing an oxide used for forming a ferrite material with water and optionally a dispersant, then grinding, and granulating and drying a resulting product;
(b) adding a granular powder obtained in (a) into a pre-sintering furnace for pre-sintering to remove CO₃²⁺ in the granules, and carrying out a preliminary pre-reaction; and
(c) pulverizing a product pre-sintered in (b) and mixing the product with a doping oxide, adding water and optionally the dispersant, and fully grinding and drying, thereby obtaining a magnetic material powder.

In an implementation, the method further comprises:
(d) preparing a laminated inductor body from the magnetic material powder obtained in (c) and then sintering the laminated inductor body.

In an implementation, the oxide used for forming the ferrite material comprises Fe₂O₃ and one or more of NiO, Mn₃O₄, CuO, and ZnO as an additive.

In an embodiment, step (a) comprises adding Fe₂O₃ and one or more of NiO, Mn₃O₄, CuO, and ZnO powders as an additive into a ball mill, fully stirring and mixing, and then carrying out spray drying by means of a spray granulator.

In an implementation, steps (a) and (c) are performed by means of a ball mill.

In an implementation, the dispersant in step (a) comprises an alcohol dispersant, such as PEG 400.

In an implementation, step (c) involves carrying out spray drying by means of a spray granulator.

In an implementation, step (d) is performed by means of tape casting.

### Advantageous Effect

According to the present invention, by adding specific doping oxide particles on the grain boundaries of the crystal structure of the magnetic material, the grain boundary resistance at low sintering temperatures can be improved and the proportion of a non-magnetic material can be minimized.

In addition, by doping the oxide particles, the sintering temperature of the ferrite material can be reduced, for example, to 890°C or lower, and a higher surface resistance can also be obtained. After the surface resistance is increased, equivalent resistance at high frequencies can be increased, and the impedance at high frequencies can also be increased. At the same time, the increased surface resistance also provides higher reliability for circuit design, allowing for a more compact circuit layout without causing a short circuit in the entire product when it is powered on.

In addition, the multilayer inductor of the present invention can implement excellent magnetic properties or magnetic flux density by comprising the magnetic material of the present invention.

### BRIEF DESCRIPTION OF THE DRAWINGS

The drawings described in the present invention are for illustrative purposes only of selected embodiments instead of all possible implementations, and are not intended to limit the scope of the present invention.
FIG. 1 is a schematic cross-sectional view of a commonly used multilayer inductor structure;
FIG. 2 is a schematic view of the microstructure of a magnetic material of the present invention;
FIG. 3 is an SEM image of the microstructure of a magnetic material prepared in Embodiment 1 of the present invention;
FIG. 4 is an EPMA image of the magnetic material prepared in Embodiment 1 of the present invention;
FIG. 5 is an inductance-frequency curve obtained by performing an electrical test on devices prepared in Embodiment 1 and Comparative Examples 1 and 2 of the present invention;
FIG. 6 is an impedance-frequency curve obtained by performing an electrical test on the devices prepared in Embodiment 1 and Comparative Examples 1 and 2 of the present invention; and
FIG. 7 is a current-inductance curve obtained by performing an electrical test on the devices prepared in Embodiment 1 and Comparative Examples 1 and 2 of the present invention.

### DETAILED DESCRIPTION

Hereinafter, the present invention will be described in more detail.

It should be understood that the terms used in the specification and the claims may be construed, on the basis of the principle that the inventor may properly define the terms, as having meanings consistent with their meanings in the context of the relevant art and the technical idea of the present invention. The terms used in the specification are used only to explain exemplary implementations, and are not intended to limit the present invention.

It should be further understood that for the terms "comprise," "include," or "have", when used in this specification, specify the presence of stated features, numbers, steps, elements, or combinations thereof, but do not preclude the presence or addition of one or more other features, numbers, steps, elements, or combinations thereof.

Herein, in describing the structure of elements with reference to the drawings, when describing the positional relationship of a certain component, "upper", "lower", "upper layer", "lower layer", etc., refer to the relative positional relationship of the component, and are not limited to the structure shown in the drawings.

A multilayer inductor of the present invention will be specifically described below.

First of all, referring to FIG. 1, a schematic cross-sectional view of a common multilayer inductor structure in the art is shown. The multilayer inductor 100 includes a plurality of magnetic layers 110, and a plurality of metal electrode tracks 120 formed on the plurality of magnetic layers.

The material of the magnetic layer may be a magnetic material, specifically a magnetic ceramic material, namely, a ferrite material. For example, as an embodiment, an oxide powder used for forming a ferrite may include an iron oxide powder, and a zinc oxide powder, a copper oxide powder, a nickel oxide powder, or the like, as an additive.

In general, as known in the art, commonly used ferrite materials may be classified into NiZn ferrite materials and MnZn ferrites. For example, a Cu additive may be further included in the NiZn ferrite material, thereby changing the formation mechanism of an NiZn ferrite phase and reducing the formation temperature of a spinel phase.

Therefore, in one implementation of the present invention, a ferrite material includes, in addition to Fe₂O₃, at least one selected from Mn₃O₄, NiO, CuO, and ZnO as an additive. Preferably, the ferrite material is an NiCuZn ferrite, with a chemical formula of NiCuZnFe₂O₄.

In a specific implementation, when the ferrite material is an NiCuZn ferrite, based on the total weight of an oxide used for forming the ferrite material, the content of Fe₂O₃ may be 62 wt% to 65 wt%; the content of NiO may be 10 wt% to 13 wt%; the content of ZnO may be 19 wt% to 22 wt%; and the content of CuO may be 2 wt% to 5 wt%.

In addition, a small amount of an Mn additive may be added to the NiCuZn ferrite to improve Bs and Tc. Thus, in a specific embodiment, based on the total weight of the oxide used for forming the ferrite material, the content of Fe₂O₃ may be 62 wt% to 65 wt%; the content of NiO may be 10 wt% to 13 wt%; the content of ZnO may be 19 wt% to 22 wt%; the content of CuO may be 2 wt% to 5 wt%; and the content of Mn₃O₄ may be 0 wt% to 1 wt%, preferably 0.1 wt% to 1 wt%.

In addition, metal electrodes include silver (Ag), platinum (Pt), palladium (Pd), copper (Cu), gold (Au), nickel (Ni), or an alloy thereof, or a composite thereof.

In the present invention, a magnetic material of a magnetic layer is formed by sintering an oxide used for forming a ferrite material and a doping oxide, and is characterized in that the magnetic material has a crystal structure, the doping oxide is distributed on grain boundaries of the crystal structure in a doped phase, and the content of the doping oxide is 5 wt% or less based on the total weight of the magnetic material.

In an implementation, the doping oxide includes silicon dioxide, bismuth oxide, optionally calcium oxide, or a combination thereof. Preferably, the doping oxide includes silicon dioxide and bismuth oxide.

FIG. 2 shows a schematic view of the microstructure of the magnetic material of the present invention. Referring to FIG. 2, the magnetic material has a plurality of magnetic grains or crystalline phases 210. The doped phase 220 of the doping oxide described above is formed at the grain boundaries between the grains or crystalline phases 210. The grains or crystalline phases 210 are formed from the ferrite material described above, e.g., an NiCuZn ferrite crystalline phase, while the doped phase 220 is formed from the doping oxide described above.

Here, in general, since the doped phase 220 is formed at the grain boundaries, under the action of elements such as Si, Bi, and Ca, grain boundary elements can affect the formation of a ferrite when the temperature rises, reducing the sintering temperature; and when the temperature drops, the grain boundary elements can precipitate in the grain boundaries to form a high-resistivity grain boundary phase.

Specifically, based the total weight of the oxide used for forming the ferrite material, the preferred added amounts or contents of the doping oxide are: SiO₂: 0.01 wt% to 0.15 wt%; Bi₂O₃: 0.1 wt% to 3 wt%; and CaO: 0 wt% to 1.5 wt%. Preferably, the content of SiO₂ may be 0.01 wt% to 0.12 wt%, 0.02 wt% to 0.10 wt%, or 0.03 wt% to 0.08 wt%; the content of Bi₂O₃ may be 1 wt% to 2.5 wt%, 1.5 wt% to 3 wt%, or 1 wt% to 2 wt%; and the content of CaO may be 0 wt% to 1 wt%, or 0.5 wt% to 1.5 wt%.

When the content of the doping oxide exceeds the upper limit values defined above, it cannot bring about a further gain in effect, but rather causes a deterioration in the properties of the obtained magnetic material, such as inductance, impedance, etc., at high frequencies.

The influences of the doping oxide are as follows. For example, adding an appropriate amount of Bi₂O₃ to an NiZn ferrite can accelerate the ion diffusion rate at lower sintering temperatures and promote the grain growth. Moreover, material modification is implemented by changing the morphology of the magnetic crystal grains via the fluxing action of Bi₂O₃ and introducing a new grain boundary phase at the microstructure level.

SiO₂ can form iron silicate with iron oxide during sintering of a ferrite, and oxygen is generated. Iron silicate has a melting point of only 1150°C, and can thus be used as a flux. Meanwhile, the addition of SiO₂ and Bi₂O₃ in the form of SiO₂·Bi₂O₃ can effectively reduce the sintering temperature of the NiZn ferrite to 890°C, and can also broaden the use frequency band of the ferrite and increase the cut-off frequency.

At the same time, SiO₂ and CaO can also form a SiO₂·CaO molten glassy phase, and the firing temperature can also be reduced. During the sintering process, the above-described SiO₂·Bi₂O₃ and SiO₂·CaO are precipitated in the grain boundaries during the cooling process, thereby forming a high-resistance compound in the grain boundaries. Therefore, the addition of SiO₂, Bi₂O₃, and optionally CaO can both reduce the sintering temperature and increase the grain boundary resistance.

In another aspect, the present invention provides a method for preparing the magnetic material, including the following steps:
(a) mixing an oxide used for forming a ferrite material with water and optionally a dispersant, then grinding, and granulating and drying a resulting product;
(b) adding a granular powder obtained in (a) into a pre-sintering furnace for pre-sintering to remove CO₃²⁺ in the granules, and carrying out a preliminary pre-reaction;
(c) pulverizing a product pre-sintered in (b) and mixing the product with a doping oxide, adding water and optionally the dispersant, and fully grinding and drying, thereby obtaining a magnetic material; and optionally
(d) preparing a laminated inductor body from the magnetic material powder obtained in (c). Then, sintering may be carried out.

In the art, sintering is generally carried out at a high temperature of 930°C to 950°C. However, in the present invention, the sintering temperature can be reduced to, for example, 890°C or lower by means of the above-described action of the doping oxide, and thus the multilayer inductor of the present invention can be obtained by co-firing the inductor core and a metal track such as silver.

For example, in an implementation, the method is performed as follows:
(a) mixing Fe₂O₃, NiO, CuO, ZnO, and optionally Mn₃O₄ with water, adding a dispersant (PEG 400), fully stirring and mixing, and then carrying out spray drying by means of a spray granulator;
(b) adding the spray-dried granular powder to a pre-sintering furnace for pre-sintering, for example, at 700°C for 2 hours, to remove CO₃²⁺ from the granules, and carrying out a preliminary pre-reaction;
(c) adding the pre-sintered powder into a ball mill jar while adding doping oxides SiO₂, Bi₂O₃, optionally CaO or CaCO₃, optionally the dispersant and water, then fully grinding, and carrying out spray drying by means of the spray granulator; and
(d) forming a cast sheet from the obtained powder by means of tape casting, and then preparing a monolithic high-impedance magnetic bead by means of lamination; and subsequently, carrying out firing under an air atmosphere, for example, sintering at 890°C for 1 to 3 hours, preferably 2 hours.

Step (a) is performed by means of ball grinding and mixing, conditions thereof are that mixing is carried out at room temperature for 4 to 8 hours, and the function thereof is mainly to mix powder.

The conditions of spray drying in steps (a) and (c) are that the temperature at an air outlet is controlled to be about 100°C.

In addition, pulverization may be carried out by means of a general ball milling method, and a target particle size thereof is D₅₀ = 1.0 to 1.3 µm.

Here, the ranges of the usage amounts of Fe₂O₃ and the additives NiO, MnO, CuO, ZnO powder, etc., are as described above for the magnetic material. In step (c), CaO may be replaced by CaCO₃, and CaCO₃ may be converted into CaO during sintering to provide a Ca source.

In an implementation, the dispersant in step (a) includes, for example, PEG 400, which has the function of implementing uniform mixing of mixed materials.

In steps (a) and (c), the usage amount of water used for mixing is not particularly limited as long as the amount used enables the mixture to be ground. For example, in a specific embodiment, the usage amount of water may be 30 wt% based on the total weight of the obtained mixture, that is, the content of solids in the mixture may be 70 wt%.

In addition, in step (d), the temperature of the tape casting is about 70°C to 90°C, for example, 80°C.

In addition, the present invention further provides a multilayer inductor, which includes a plurality of magnetic layers and metal electrode tracks formed on the magnetic layers, the magnetic layers including the magnetic material for the magnetic core of the multilayer inductor described above.

As described above, since the magnetic material of the present invention has a higher surface resistance, the multilayer inductor of the present invention can increase the equivalent resistance at high frequencies, and can also increase the impedance at high frequencies; moreover, the improved surface resistance also provides higher reliability for circuit design, so that the multilayer inductor of the present invention may be applied to various fields.

### Embodiments

Hereinafter, the present invention will be explained in detail with reference to embodiments. However, the embodiments of the present invention may be modified into various other types, and the scope of the present invention should not be limited to the implementations described below. The embodiments of the present invention are provided to completely explain the present invention to those having ordinary knowledge in the art.

The percentages referred to in the embodiments are based on mass, unless otherwise specified. Moreover, the raw materials and equipment information involved in the embodiments are as follows:
Fe₂O₃: analytical reagent grade, Fe₂O₃ ≥ 99.5%
NiO: analytical reagent grade, NiO ≥ 99.7%
Mn₃O₄: analytical reagent grade, Mn₃O₄ ≥ 99.5%
CuO: analytical reagent grade, CuO ≥ 99.7%
ZnO: analytical reagent grade, ZnO ≥ 99.7%
SiO₂: analytical reagent grade, SiO₂ ≥ 99.9%, nano-SiO₂
Bi₂O₃: analytical reagent grade, Bi₂O₃ ≥ 99.7%
CaCO₃: analytical reagent grade, CaCO₃ ≥ 99.7%
Dispersant: PEG 400 polyvinyl alcohol
Water: deionized water, conductivity less than 0.1 µS/cm
Ball mill: planetary ball mill, conventional experimental machine
Spray granulator: small spray granulator, conventional experimental machine
Electron scanning microscope: ZEISS EVO MA10, Zeiss, Germany
Electron probe (EPMA) test equipment: JEOLJXA-8230

### Embodiment 1

Based on a ferrite material to be prepared, 66 wt% (147.84 g) of Fe₂O₃, 9 wt% (20.16 g) of NiO, 1 wt% (2.24 g) of Mn₃O₄, 4 wt% (8.96 g) of CuO, and 20 wt% (44.8 g) of ZnO powder were added to a ball mill jar, and 400 g of water and 1 g of a dispersant (PEG 400) were further added, followed by ball mill mixing (4 h, room temperature) and spray drying (2 h, 100°C) by means of a spray granulator. Then, the spray-dried granular powder was added into a pre-sintering furnace for pre-sintering.

Next, based on the total weight of the pre-sintered ferrite material, 0.08 wt% (0.18 g) of SiO₂, 1 wt% (2.24 g) of Bi₂O₃, and 1 wt% (0.67 g) of CaCO₃ were added as doping oxides, and ball grinding (10 h, room temperature) and spray drying (2 hours, room temperature) were carried out, thereby forming a desired magnetic material powder.

Then, a laminated inductor was prepared from the obtained magnetic material powder by means of tape casting, and was co-sintered (890°C, 2 hours) with Ag tracks to obtain a multilayer inductor of Embodiment 1, which has the basic structure shown in FIG. 1.

The magnetic core of the obtained multilayer inductor was subjected to electron scanning, and an SEM image thereof is shown in FIG. 3, and it can be seen that the magnetic core of the obtained multilayer inductor has a uniform crystalline phase structure.

The element distribution of the magnetic core was analyzed using EPMA technology to obtain the image shown in FIG. 4. It can be seen that the doping elements (Ca, Si, and Bi) are distributed as a doped phase at the grain boundaries of the crystalline phase structure, as shown in the white portion of FIG. 4.

### Comparative Example 1

Based on a ferrite material to be prepared, 66 wt% (147.84 g) of Fe₂O₃, 9 wt% (20.16 g) of NiO, 1 wt% (2.24 g) of Mn₃O₄, 4 wt% (8.96 g) of CuO, and 20 wt% (44.8 g) of ZnO powder were added to a ball mill jar, and 400 g of water and 1 g of a dispersant (PEG 400) were further added, followed by ball mill mixing (4 h, room temperature) and spray drying (2 h, 100°C) by means of a spray granulator. Then, the spray-dried granular powder was added into a pre-sintering furnace for pre-sintering.

Next, ball grinding (10 h, room temperature) and spray drying (2 hours, room temperature) were carried out, thereby forming a desired magnetic material powder.

Then, a laminated inductor was prepared from the obtained magnetic material powder by means of tape casting, and was co-sintered (890°C, 2 hours) with Ag tracks to obtain a multilayer inductor of Comparative Example 1.

### Comparative Example 2

Based on a ferrite material to be prepared, 66 wt% (147.84 g) of Fe₂O₃, 9 wt% (20.16 g) of NiO, 1 wt% (2.24 g) of Mn₃O₄, 4 wt% (8.96 g) of CuO, and 20 wt% (44.8 g) of ZnO powder were added to a ball mill jar, and 400 g of water and 1 g of a dispersant (PEG 400) were further added, followed by ball mill mixing (4 h, room temperature) and spray drying (2 h, 100°C) by means of a spray granulator. Then, the spray-dried granular powder was added into a pre-sintering furnace for pre-sintering.

Next, based on the total weight of the pre-sintered ferrite material, 0.2 wt% (0.4 g) of SiO₂, 1.5 wt% (3 g) of Bi₂O₃, and 2 wt% (4 g) of CaCO₃ were added as doping oxides, and ball grinding (10 h, room temperature) and spray drying (2 hours, room temperature) were carried out, thereby forming a desired magnetic material powder.

Then, a laminated inductor was prepared from the obtained magnetic material powder by means of tape casting, and was co-sintered (890°C, 2 hours) with Ag tracks to obtain a multilayer inductor of Embodiment 2.

### Test Example:

In this test example, the impedance was tested using an impedance test instrument 4396, and the inductance was tested using an Agilent 4991 network analyzer.

The multilayer inductors obtained in Embodiment 1 and Comparative Examples 1 to 2 were tested, and the results are shown in FIGS. 5 to 7.

By determining additives to minimize non-magnetic components in the magnetic core, it can be seen from FIGS. 5 to 7 that:
1. By means of the function of Si, Ca, and Bi to promote low-temperature firing, the compactness of the product itself is improved, that is, from 4.98 g/cm³ to 5.2 g/cm³, thereby improving Bs, that is, the maximum magnetic flux density is improved from 0.3 tesla to 0.35 tesla, thereby improving the DC superposition property of the product, which can be seen from the current-inductance diagram (FIG. 7), wherein when the current is > 1A, the inductance decreases slowly, indicating that the superposition property becomes better;
2. At the same time, the inductance at high frequencies is improved by means of the high grain boundary resistance formed by SiO₂·CaO and SiO₂·Bi₂O₃ after cooling, so the inductance at high frequencies can also be improved; and
3. After the sintering temperature is lowered, the crystal grain size is reduced, which is also helpful for increasing the inductance at high frequencies, thereby forming the effect of improving the impedance.

In addition, it can be confirmed that when the doping element Si, Bi, or Ca of the present invention is not contained, the sintering temperature is significantly increased since the doped phase is not formed at the grain boundaries. Moreover, referring to FIGS. 5 and 6, it can be seen that the inductance material obtained in Comparative Example 1 has the lowest impedance and the lowest inductance, which is significantly inferior to Embodiment 1 of the present invention.

Furthermore, by comparing Embodiment 1 and Comparative Example 2, it can be seen that if the doping element of the present invention is added in excess, it can be seen from an inductance-frequency curve (FIG. 5) that the inductance can be improved, but the inductance at high frequencies (near 100 MHz) is not improved (Comparative Example 2). In contrast, the inductance of Embodiment 1 maintains a higher value even at a high frequency. Further, it can be seen from an impedance-frequency curve (FIG. 6) that the impedance of Comparative Example 2 is improved compared to Comparative Example 1, but the impedance increase value is far inferior to that of Embodiment 1. In addition, it can be seen from a current-inductance curve (FIG. 7) that the improved inductance does not improve the DC-Bias characteristic well. Thus, it is also demonstrated that the doping elements of the present invention, such as Si, Bi, Ca, etc., should be maintained within the ranges defined above.

Those skilled in the art will appreciate that many modifications and other implementations of the technical solutions described herein are possible in light of the teachings presented in the foregoing specification and the associated drawings. Therefore, it is to be understood that the present invention is not to be limited to the specific implementations disclosed and that all modifications and other implementations are intended to be included within the scope of the appended claims.

## Claims

1. A magnetic material for a magnetic core of a multilayer inductor, the magnetic material being formed by sintering an oxide used for forming a ferrite material and a doping oxide, and being **characterized in that** the magnetic material has a crystal structure, the doping oxide is distributed on grain boundaries of the crystal structure in a doped phase, and the content of the doping oxide is 5 wt% or less based on the total weight of the magnetic material.

2. The magnetic material according to claim 1, wherein the doping oxide comprises silicon dioxide, bismuth oxide, optionally calcium oxide, or a combination thereof.

3. The magnetic material according to claim 1, wherein the ferrite material comprises Fe₂O₃, and at least one selected from Mn₃O₄, NiO, CuO, and ZnO as an additive.

4. The magnetic material according to claim 1, wherein based on the total weight of the oxide used for forming the ferrite material, the ferrite material comprises the following components:
Fe₂O₃ : 62 wt% to 65 wt%;
NiO: 10 wt% to 13 wt%;
ZnO: 19 wt% to 22 wt%;
CuO: 2 wt% to 5 wt%; and
Mn₃O₄ : 0 wt% to 1 wt%.

5. The magnetic material according to claim 1, wherein based on the total weight of the oxide used for forming the ferrite material, the content of the doping oxide is:
SiO: 0.01 wt% to 0.15 wt%;
Bi₂O₃: 0.1 wt% to 3 wt%; and
CaO: 0 wt% to 1.5 wt%.

6. A method for preparing the magnetic material of any one of claims 1 to 5, the method comprising the following steps:
(a) mixing an oxide used for forming a ferrite material with water and optionally a dispersant, then grinding, and granulating and drying a resulting product;
(b) adding a granular powder obtained in (a) into a pre-sintering furnace for pre-sintering to remove CO₃²⁺ in the granules, and carrying out a preliminary pre-reaction; and
(c) pulverizing a product pre-sintered in (b) and mixing the product with a doping oxide, adding water and optionally the dispersant, and fully grinding and drying, thereby obtaining a magnetic material powder.

7. The method according to claim 6, further comprising:
preparing a laminated inductor body from the magnetic material powder obtained in (c) and then sintering the laminated inductor body.

8. The method according to claim 6, wherein:
the dispersant in steps (a) and (c) comprises an alcohol dispersant.

9. A multilayer inductor, comprising a plurality of magnetic layers and metal electrode tracks formed on the magnetic layers, the magnetic layers comprising the magnetic material of any one of claims 1 to 5.

10. The multilayer inductor according to claim 9, wherein the metal electrodes comprise silver (Ag), platinum (Pt), palladium (Pd), copper (Cu), gold (Au), nickel (Ni), or an alloy thereof, or a composite thereof.
